

H. V. LINDERMAN.  
METHOD OF MANUFACTURING RAIL BONDS.  
APPLICATION FILED SEPT. 29, 1919.

1,369,927.

Patented Mar. 1, 1921.



Witness

S. J. Mathis

By

Inventor  
Harry V. Linderman

Signature

Attorney

# UNITED STATES PATENT OFFICE.

HARRY V. LINDERMAN, OF MANSFIELD, OHIO, ASSIGNOR TO THE OHIO BRASS COMPANY, OF MANSFIELD, OHIO, A CORPORATION OF NEW JERSEY.

## METHOD OF MANUFACTURING RAIL-BONDS.

1,369,927.

Specification of Letters Patent.

Patented Mar. 1, 1921.

Original application filed April 23, 1919, Serial No. 292,132. Divided and this application filed September 29, 1919. Serial No. 327,080.

To all whom it may concern:

Be it known that I, HARRY V. LINDERMAN, a citizen of the United States of America, residing at Mansfield, in the county of Richland and State of Ohio, have invented certain new and useful Improvements in Methods of Manufacturing Rail-Bonds, of which the following is a specification.

10 My invention relates to the method of manufacturing that class of bond which is adapted to be secured to the conductor rail by means of a concentrated heating flame of very high intensity.

15 I have found that the requirements of a bond of this character when it is desired to apply it to the rail by means of a ferrous attaching metal requires certain refinements in its construction not present in bonds 20 adapted to be applied by a copper, bronze or brass attaching metal and the method of carrying out the construction of such a bond is of great importance.

It is not difficult to construct a bond to be 25 applied by a concentrated heating flame of high intensity when the attaching metal consists of copper, bronze or brass, etc., but when it is desired to use a ferrous attaching metal and the body of the bond and terminal 30 are composed of copper, a metal having a high electrical conductivity, it is found that the difference in temperature between the ferrous metal and the copper terminal is so great that the copper terminal is liable to 35 become fused or fluid and run before the ferrous attaching metal has reached a molten condition; and another difficulty is that the molten copper and iron do not properly unite or alloy under the ordinary conditions 40 of melting such as is present in the application of a bond.

The object of using a ferrous attaching metal is that in itself it is cheaper and more economical than copper, bronze or brass and 45 at the same time its mechanical strength is much greater than copper or the copper alloys.

To bring about a construction to meet the above conditions and to produce a bond 50 which will have high electrical conductivity and other features set forth hereinafter, requires a method of manufacture which com-

prises certain features of novelty herein-after described and shown in the accompanying drawings and these features of novelty are not only hereinafter described and shown in the accompanying drawings but are more particularly pointed out in the claims.

This application forms a division of my copending application, Serial No. 292,132 filed April 23, 1919.

In the drawings:

Figure 1 shows the stranded body portion of my bond.

Fig. 2 shows an end view of Fig. 1.

Fig. 3 shows the body of my bond after it has had its end upset and compressed into a more compact mass.

Fig. 4 is an end view of Fig. 3.

Fig. 5 is a section on the line 5—5 of Fig. 3 and shows how the face of the body and sleeve have been altered, compressed together and reinforced and the voids between the strands which were present in Fig. 2 have been eliminated.

Fig. 6 shows a sectional view on the line 6—6 of Fig. 3 and shows the same condition as in Fig. 2, indicating that the operation of upsetting the body and a portion of the sleeve has left unchanged or practically so, a portion of the body and sleeve.

Fig. 7 shows a side elevation view of the body and sleeve after it has been heated and further compressed to bring the strand members into a close and intimate union with each other and practically making a solid homogeneous terminal.

Fig. 8 shows an end view of Fig. 7.

Fig. 9 is a sectional view on the line 9—9 of Fig. 7 and shows how the compression of the terminal has caused the individual strands to lose their identity and the cross section area reduced, all as compared with the structure shown in Fig. 5.

Fig. 10 is a sectional view on the line 10—10 of Fig. 7 and shows practically an unchanged condition at this point of the body and sleeve.

Fig. 11 shows a side elevation view of a partially formed casing ready to be applied to the terminal shown in Fig. 7. This casing I prefer to make of as pure a grade of iron as possible as it has particular properties which are very advantageous for a bond

of the class herein described and the requirements which it is expected to meet, although other grades of ferrous metal can be used.

Fig. 12 is an end view of Fig. 11.

5 Fig. 13 is a side view in elevation of a member which is interposed between the casing 11 and the terminal of the bond and which when subjected to a proper temperature will melt and unite the casing 11 securely to the terminal of the body member both electrically and mechanically.

Fig. 14 is an end view of Fig. 13.

Fig. 15 is an end view of the terminal shown in Fig. 7 with the casing shown in 15 Fig. 11 and the interposed attaching metal shown in Fig. 13 in a partially assembled condition.

Fig. 16 is the same view as Fig. 15 but showing the parts in a further state of completion in which the case or casing has been folded down into position against all sides 20 of the terminal member.

Fig. 17 shows the bond in a completed condition in which the casing has been securely united to the terminal.

Fig. 18 is an end view of Fig. 17.

Fig. 19 shows a terminal of my bond secured to one face of a rail as is used in practice. It is however, adapted to be 30 applied to other faces or surfaces of the rail as well as that shown.

In the method of construction of my improved bond I first prepare a length of stranded cable 1 as shown in Fig. 1 and 35 upon each end provided with a terminal I position a sleeve 2 so that in the finished bond this sleeve will project partially out of the terminal proper in the finished bond. The object of this sleeve is to protect the 40 strands of the body 1 at the point where they enter the terminal, from mechanical injury and also from heat used in securing the casing to the body terminal.

In order to secure a core for the terminal 45 of my bond which shall be of high conductivity, I utilize the end portions of the body member 1 and in order to do so I find it advisable to increase the amount of stranded ends in the terminal in order to be 50 able to produce a solid core for the terminal which is preferable but not necessary, and in order to do this I upset the end of the body 1 in such a manner as to produce an enlarged cross-section of compacted and 55 closely compressed strands and in which the air spaces between the strands as originally produced are practically eliminated. When upsetting the ends of the body 1, I include in the upset portion, part of the 60 sleeve member 2 in order that it may become a part of the completed terminal and be retained at the point where the flexible body projects from the member 11 for the purpose above stated.

65 I now have as shown in Fig. 3 a flexible

body 1 with an upset, compressed and compacted terminal 3 formed out of the ends of the body 1 and a sleeve or collar 2 united therewith at the point where the flexible portion ends and the compressed upset portion begins.

I now heat the ends 3 of the body and bring them to a heat sufficient under pressure to cause the individual strands of the terminal 3 to lose their identity and become 75 further compacted to a practically solid structure and under some conditions actually welded together; especially is this so when the strands have been sufficiently compacted together to eliminate the air films between the strand surfaces, thereby preventing oxidation, and the heat has been sufficiently great to properly soften the strand surfaces. The body and terminal thus treated will produce the member shown in 80 Figs. 7, 8, 9 and 10.

I now have formed the flexible conducting portion of my bond with an integrally formed terminal member which acts as a conducting core in the completed terminal 90 of my bond and this conducting core tends to make the terminal of almost equal conductivity throughout its length and at the same time there is no joint or union between the body 1 and the solid compacted 95 core 4.

The complete member as shown in Fig. 7 would be suitable to be applied to a rail by means of a welding metal of copper, bronze or brass, etc., but is not adapted to be secured to the rail by means of a ferrous welding or attaching metal; therefore I secure by welding or brazing to one or more faces of each terminal a casing or coating composed of iron, steel, Monel metal, etc., which 105 has a melting temperature practically the same or in excess of that of the attaching metal.

Where I use iron I prefer to use a material which is practically pure, namely not 110 less than 99.8% as such metal offers several advantages; namely, its electrical conductivity is very high compared with ordinary iron or steel which is high in carbon, silicon, manganese, sulfur, etc., and it is found to be 115 practically rustproof which is a very important item in connection with rail bonds. In order to secure these advantages I prefer to use what is known as Armco-iron having a higher electrical conductivity and 120 greater anti-corroding properties.

In order to prepare the casing 5 shown in Fig. 11, I use the iron in sheet form and bend it into shape shown in Fig. 11 and Fig. 12 or other suitable shapes to fit the 125 terminal 4.

I then form up a similar shaped member 6 shown in Figs. 13 and 14 out of a material which will unite with the iron casing 5 and the copper terminal 4 when proper heat or 130

heat and pressure are applied. This material may be the ordinary brazing metal of copper-zinc base or a silver solder or brazing metal composed of silver-copper base or 5 other uniting metals of similar character.

I now assemble the parts 5 and 6 together with the terminal 4 as shown in Fig. 15 with the uniting metal 6 interposed between the terminal 4 and the casing 5. The projecting portions of the members 5 and 6 are now 10 bent over into place as shown in Fig. 16.

I now apply heat to the terminal of the bond assembled as described, sufficient to cause the attaching metal 6 to melt and unite 15 with the copper terminal 4 and the casing 5, after which I may apply pressure to bring the parts into closer relation if desired.

This completes the formation of a terminal and the result is a bond as shown in 20 Fig. 17.

There are many modifications in the production of this bond which can be made without departing from the spirit of the invention.

25 It may be found advantageous in some cases to use in connection with the attaching metal interposed between the ferrous sleeve and the bond 4, a fluxing material such as borax or boracic acid to assist in the uniting of the parts. It may under some circumstances be found an advantage to use a granulated attaching metal in place of the attaching metal in sheet form as shown in 30 Figs. 13 and 14 and when such granulated attaching metal is used it is usually mixed 35 into a paste with the borax or boracic acid and applied to the inner surface of the ferrous sleeve or the exterior surface of the bond core. This application of the granulated attaching metal and fluxing material 40 in a paste form is applied prior to the assembly of the ferrous sleeve and the bond core. Another modification may consist in applying the members 5 and 6 directly to 45 the terminal 3 as shown in Fig. 3 and then heating the same to a temperature which will melt the attaching metal as in the case of where the members 5 and 6 are applied to the terminal 4 as shown in Fig. 4 and de- 50 scribed above. This latter modification avoids the necessity of one heating but the terminal 4 is not compressed and compacted to the degree as the construction herein first described and the spaces or interstices between the strands will be filled to a degree 55 by the attaching metal.

Modifications may be made in the last 60 pressing operation referred to in that this operation may be made at the time of the final heating, that is simultaneously therewith, or it may be made immediately after the final heating and while the parts are still hot and the brazing metal in a practically fluid state.

65 A bond constructed as herein described

and applied by means of attaching metal of a ferrous character will be found to be more strongly united to the rail than a bond in which the terminal is composed of copper and in which the bond is secured to the rail 70 by means of copper, bronze, or brass, as in the latter case there is a formation of oxidized or spongy copper between the copper terminal and the bond and the copper or bronze attaching metal, and this oxidized 75 or spongy copper is very weak mechanically and permits the bond to be very easily removed from the rail, but when the attaching surface of the bond terminal is of iron, steel or Monel-metal, the union between the terminal and the attaching metal cannot be broken and the resistance of the bond against removal is dependent upon the mechanical strength of the attaching metal entirely. In Fig. 19 the rail is represented by 80 the numeral 7 and the bond terminal by the numeral 8 and the attaching metal by the numeral 9.

Having described my invention, what I claim as new herein and desire to secure by 90 Letters Patent is:—

1. The method of forming an electrical conductor comprising the steps of upsetting and compressing the component strands of a cable end cold, then heating and further 95 compacting the strands, then inclosing the upset end of the cable in a ferrous casing with a brazing metal interposed and pressing the parts firmly together, then heating the parts to a temperature at which the 100 brazing metal becomes fluid and applying pressure to the parts to unite the parts.

2. The method of forming an electrical conductor comprising the steps of upsetting and compressing the component strands of 105 a cable end cold, then heating and further compacting the strands, then inclosing the upset end of the cable in a ferrous casing with a brazing metal interposed and pressing the parts firmly together, then heating 110 the parts to a temperature at which the brazing metal becomes fluid to unite the parts.

3. The method of forming an electrical conductor comprising the steps of upsetting 115 and compressing the component strands at the end of a cable, then forming up an inclosing member having a melting point higher than that of the cable to fit the upset cable end, then forming up an inclosing member to fit the upset cable end having a lower melting point than the cable, then assembling the cable and inclosing members with the last mentioned inclosing member interposed between the first mentioned inclosing member and the upset cable end, then heating the parts thoroughly and to a temperature at which the interposed member becomes fluid and then applying pressure to 120 the parts.

4. The method of forming an electrical conductor comprising the steps of upsetting and compacting the ends of the individual members forming a stranded conductor, then inclosing the upset ends in a ferrous casing having interposed brazing metal therebetween, then heating the parts to a point at which the brazing metal is thoroughly fluid.
5. The method of forming an electrical conductor comprising the steps of upsetting and compacting the ends of the individual members forming a stranded conductor, then inclosing the upset ends in a ferrous casing having interposed brazing metal therebetween, then heating the parts to a point at which the brazing metal is thoroughly fused and simultaneously applying pressure.
6. The method of forming an electrical conductor comprising the steps of upsetting and compacting the end of a stranded cable into a practically homogeneous and solid structure, then inclosing the upset end of the cable in a ferrous casing, then heating the parts to a point at which they will unite and simultaneously applying pressure.
7. The method of forming an electrical conductor which consists of heating, upsetting and compacting the component strands of a cable end into a practically homogeneous and solid structure, then applying a plate of ferrous metal to the upset cable end with interposed brazing metal, then heating and compressing the parts to unite them together.
8. The method of forming an electrical conductor which comprises the steps of up-
- setting and compacting the end strands of a cable, then applying a plate of ferrous metal with interposed brazing metal, then heating and compressing the above parts to unite them together.
9. The method of forming an electric conductor comprising the steps of upsetting and compressing the component strands of a cable end cold, then heating and further compacting the strands, then inclosing the upset end of the cable in a ferrous casing with brazing metal interposed, then heating the parts to a temperature at which the brazing metal becomes fluid and applying pressure to the parts to unite the parts.
10. The method of forming an electric conductor comprising the steps of upsetting and compacting the end of the individual members forming a stranded conductor, then inclosing the upset end in a ferrous casing having interposed brazing metal therebetween, then heating the parts to a point at which the brazing metal is fused and then applying pressure to the part while still hot.
11. The method of forming an electrical conductor comprising the steps of upsetting and compressing the component strands of a cable end, then heating and further compacting the strands, then inclosing the upset end of the cable in a ferrous casing with a brazing metal interposed, and pressing the parts firmly together, then heating the parts to a temperature at which the brazing metal becomes fluid to unite the parts.

In testimony whereof I affix my signature.  
HARRY V. LINDERMAN.